

# United States Patent Office

2,947,640

Patented Aug. 2, 1960

1

2,947,640

## PROCESS FOR THE TREATMENT OF TRACING PAPERS TO MAKE THEM READILY ERASABLE UPON

Maurice J. B. Ladeuze, 28 Rue Pre-Gentil, Rosny-sur-Bois, France, and Pierre Toni, 6 Villa des Buissonets, Chemin du Buisson, Champigny, France

No Drawing. Filed Sept. 2, 1958, Ser. No. 758,567

Claims priority, application France Feb. 21, 1958

2 Claims. (Cl. 106—2)

The present invention has for its object the provision of a process for the treatment of tracing papers permitting the very rapid erasure of lines made with Chinese ink or greasy ink on the surface treated. This process has the advantage of permitting also the erasure of all traces of pencil (by means of a soft rubber, known as a pencil rubber) without attacking the ink lines and without altering the quality of the surface treated, on which the ink lines can be rapidly erased in the dry without the employment of a scraper by the simple rubbing of a pad of metal wadding or similar material which is very slightly abrasive; on the surface thus erased upon, new lines can be made directly without re-finishing or resizing and the operation can be carried out a number of times at the same place.

The process consists essentially in covering the surface to be treated with a solution, for filling the pores of the tracing paper, which is practically colourless, and in allowing it to dry; the said coating reduces the penetration of the ink to that necessary for a sufficient grip in practice. Moreover, this treatment gives to the surface of the tracing paper a greater regularity, permitting to obtain lines of greater clarity. It will be understood that this covering can be made either on finished tracing paper, or in the last stage of manufacture, and on one or both surfaces of the tracing paper.

The number of substances, of solvents, of plasticizers, of varnishes, which lend themselves to the composition of this filling solution is only limited in practice by the inconveniences which certain of them would present, either in application of the solution, its penetration and its drying, or in the adherence of pencils and inks used later on the surfaces treated.

The formulae indicated below are given only by way of non-limiting example, as having given satisfactory results on various samples of tracing paper commercially available:

### Formula 1

Parts by weight

|                               |    |
|-------------------------------|----|
| (a) Alcohol (ethyl or propyl) | 43 |
| (b) Sodium carbonate          | 4  |

2

Parts by weight

|                          |     |
|--------------------------|-----|
| (c) Stearine             | 4   |
| (d) Benzene              | 26  |
| (e) Ethylamine           | 9   |
| (f) Ethanolamine         | 9   |
| (g) Oleic acid (° Baumé) | 5   |
|                          | 100 |

10 The products (a) (b) and (c) are heated on a water bath whilst being mixed. Then the other products are added. There is obtained a liquid which can be made pasty or solid by the addition of stearic acid.

### Formula 2

Parts by weight

|                                                   |     |
|---------------------------------------------------|-----|
| (a) Alcohol (ethyl or propyl)                     | 35  |
| (b) Benzene                                       | 35  |
| (c) Morpholine (C <sub>4</sub> H <sub>9</sub> ON) | 10  |
| (d) Stearic acid (° Baumé)                        | 11  |
| (e) Glycerine                                     | 6   |
| (f) Borax                                         | 3   |
|                                                   | 100 |

25 The mixture constitutes a gelatinous product which can be made more liquid or more solid by respectively diminishing or increasing the proportion of stearic acid.

We claim:

1. A preparation for treating tracing paper, so as to fill the pores thereof and reduce ink penetration, including the following constituents:

|                  |    |
|------------------|----|
| Ethyl alcohol    | 43 |
| Sodium carbonate | 4  |
| Stearine         | 4  |
| Benzene          | 26 |
| Ethylamine       | 9  |
| Ethanolamine     | 9  |
| Oleic acid       | 5  |

2. Tracing paper having a surface treated with the preparation claimed in claim 1.

### References Cited in the file of this patent

#### UNITED STATES PATENTS

|              |               |                |
|--------------|---------------|----------------|
| 45 149,449   | Dean          | Apr. 7, 1874   |
| 1,073,129    | Horn          | Sept. 16, 1913 |
| 1,872,662    | Brathing      | Aug. 23, 1932  |
| 1,996,858    | Davidson      | Apr. 9, 1935   |
| 2,005,113    | Smiley        | June 18, 1935  |
| 2,018,638    | Driessen      | Oct. 22, 1935  |
| 50 2,205,042 | Lenher et al. | June 18, 1940  |
| 2,267,240    | Kummel        | Dec. 23, 1941  |

### OTHER REFERENCES

55 Witham: "Modern Pulp and Paper Making" (1942), 71 and 76.